

(No Model.)

C. L. COFFIN.

METHOD OF WELDING METALS BY ELECTRICITY.

No. 423,732.

Patented Mar. 18, 1890.



Witnessed  
Cyrus L. Coffin  
G. H. Anderson.

Inventor  
Charles L. Coffin,

# UNITED STATES PATENT OFFICE.

CHARLES L. COFFIN, OF DETROIT, MICHIGAN.

## METHOD OF WELDING METALS BY ELECTRICITY.

SPECIFICATION forming part of Letters Patent No. 423,732, dated March 18, 1890.

Application filed November 12, 1889. Serial No. 330,099. (No model.)

*To all whom it may concern:*

Be it known that I, CHARLES L. COFFIN, of Detroit, in the county of Wayne and State of Michigan, have invented a new and useful 5 Improvement in Welding Metals by Electricity, of which the following is a specification.

My invention relates to the method of welding metals by electricity, in which the articles to be welded are connected with the poles of 10 a source of electricity; and it consists in creating an electrical resistance at the joint greater than that of the two articles to be welded, whereby the heating effect of the current is increased.

15 The drawing is a perspective of mechanism which may be used to practice my invention.

A represents a base, on which is carried a clamp N N, insulated therefrom by suitable insulating material D.

20 B represents a standard rising from base A, carrying at its upper end a head E, insulated therefrom by suitable insulating material C.

F represents a dovetail groove in head E.

H H represent the two parts of a clamp, 25 one of which is fitted with a dovetail projection to engage with and travel in groove F.

I represents a screw-shaft swiveled in a bracket J on head E and engaging with a nut tapped in a projection K on one part of 30 clamp H H.

The two parts of clamps N N and H H are drawn together by screw-bolts, as indicated in the drawing.

G and M represent the articles to be welded—for example, two bars of iron.

35 L represents a substance which is a conductor of electricity, but whose electrical resistance is greater than that of G and M, and for convenience L is held by an insulating- 40 handle.

P and O represent electrical conductors by which the clamps H H and N N are respectively connected with the opposite poles of a generator of electricity.

45 The operation of my invention is as follows: The articles G and M being firmly secured in the clamps H and N, the clamp H is fed down by the screw-shaft I until the ends of G and M come in contact. The electric cur-

rent is now passed through conductors P O, 50 clamps H N, and bars G M. If the electrical resistance of G M at their point of contact is sufficient to materially impede the passage of the available current, the ends of G and M will be heated; but if the electrical resist- 55 ance of G and M at their point of contact is sufficiently low to permit the ready passage of the available current no heating effect, or only slight heating effect, will be produced, and G and M cannot be welded by this 60 method. At this point my invention comes into play. The material L, which may be platinum or any conductor of electricity having a greater electrical resistance than G and M at their point of contact, is laid upon the 65 end of M, and the end of G is brought into contact with the upper surface of L. The current being turned on, L becomes heated and heats the ends of G and M. As the ends G and M become hot their electrical resist- 70 ance increases, and thus increases the heating effect of the current, until finally a welding heat is attained, and the weld is completed by pressing G against M by means of a screw-shaft I. L may be withdrawn (by 75 slightly raising G) at any time after the ends G and M become hot enough to offer sufficient resistance to the passage of the current; or, if it is a substance of little value, which will volatilize or become alloyed with the metal 80 being treated at or below a welding heat, it may be permitted to volatilize or become alloyed, and G and M then brought into contact. This process admits welding large masses by a current of insufficient power or 85 volume to heat the materials in the ordinary mode, and the interposed material L may also be used as a reducer of the local heating effect of the current by carrying the extreme heat itself and gradually bringing the mate- 90 rials to be welded to the desired heat.

What I claim as my invention, and desire to secure by Letters Patent, is—

1. The herein-described process of welding metals electrically, consisting in interposing 95 between the surfaces to be welded a conductor of greater electrical resistance than the materials being operated upon, and pass-

ing the electric heating-current through the said materials and the conductor, substantially as described.

2. The herein-described process of welding metals electrically, consisting in bringing the surfaces to be welded in contact with a conductor of greater resistance, passing heating-currents through the articles to be welded

and the interposed conductor, removing said interposed conductor and completing the weld to by pressure.

CHARLES L. COFFIN.

Witnesses:

CYRUS E. LOTHROP,  
GERTRUDE ANDERSON.